

## UNITED STATES PATENT OFFICE

NELSON J. QUINN, OF TOLEDO, OHIO, ASSIGNOR TO THE METAL CASTINGS HOLDING CORPORATION, OF CLEVELAND, OHIO, A CORPORATION OF DELAWARE

## PERMANENT MOLD

No Drawing.

Application filed November 28, 1927. Serial No. 235,398.

The present invention, relating as indicated to molds, is particularly directed to a so-called permanent, or, more accurately, a long-life, mold which may be used for the casting of metal therein. The principal object of the invention is the provision of a refractory mold which may be used for repeated castings and which shall have the desired and necessary characteristics of considerable physical strength and the ability to retain in the cast metal, or at least to prevent the transference of, heat from the molten metal at such a rate as to produce an uncommercial grain structure in the castings.

To the accomplishment of the foregoing and related ends, said invention, then, consists of the means hereinafter fully described and particularly pointed out in the claims; the following description setting forth in detail certain steps embodying the invention, such disclosed steps constituting, however, but one of the various ways in which the principle of the invention may be used.

Molten metal of various kinds has for centuries been cast in and against sand molds which have been found to be practically the only satisfactory mold up to the present time for the casting of metal in order to produce a desirable and commercial grain structure, the required smoothness of the metal, and to cause the metal to conform to and lay against the mold. The use of sand molds is based upon the porosity in the sand, i. e. quartz particles with clay, which is of course due to the openings between the particles of sand, the structure of the mold being porous and capable of withstanding the heat of the molten metal which is cast therein; and at the same time being capable of preventing, by reason of the porosity, any rapid or sudden transference of the heat from the molten metal which will produce a too sudden setting or chilling in the casting which causes the formation of an uncommercial grain structure and, in gray iron castings, extremely hard unmachinable spots. In order to form the mold from sand the latter is damped with water, rendering the particles of sand sufficiently adhesive to hold the structure together until the molten metal introduced in

the mold has set. The heat from the metal destroys the slight bond between the particles of sand, however, and the mold disintegrates and in practice, therefore, must be reformed for each casting, the sand being dumped out of the molds, remixed and retempered with a substance rendering it adhesive, such as water, before it is again ready for use.

Close attention has been paid in modern foundries to the condition of the sand which is carefully graded to produce varying degrees of porosity in the molds formed therefrom, and is tempered in many cases to a given degree of humidity before being used. The fineness of the sand, and also the amount of moisture introduced determine the porosity of the mold, and the latter, while varying considerably for different types of metals and different types of castings, must always contain a minimum amount of porosity in order to prevent the too sudden setting or chilling of the molten metal.

From studying the use and condition of sand molds I have determined that it is entirely possible to produce a permanent or non-sand mold of refractory materials united with considerable strength and having a sufficient refractoriness to withstand the temperature of the molten metal cast thereagainst, providing such material is given an effective porosity approximating that of the sand mold to be used for casting the same metal. Successful casting depends entirely upon the porosity of the molds into which the metal is cast, and porosity in turn is merely another statement of the rate of heat transference into the mold from the molten metal. Therefore, if a permanent mold of some non-sand material can be produced having the same effective rate of heat transference there is no reason why such a mold will not be clearly effective in producing sound, smooth, commercial castings of uniform grain, and in also having a life sufficient to cast a number of castings therein. After numerous experiments I have succeeded in producing such molds, in which I have incorporated the same effective rate of heat transference, or, stating the same thing in other terms, the same effective "blanketing" or insulation of the

heat in the molten metal that is present in sand molds combined with considerable mechanical strength sufficient to withstand the disintegrating effect of the molten metal and of the repeated severe changes in temperature when the metal is cast into the mold.

My improved mold may be formed of a variety of materials, providing the base material employed is sufficiently refractory to withstand the temperature of the metal for which it is to be used as a mold, and is capable of uniting with the other particles of the same material or other materials employed therewith, with a bond sufficiently strong to withstand the disintegrating effect of the casting of molten metal thereagainst, and, finally, is capable of producing a porous structure containing a multiplicity of air cells or passages to provide the retarding effect on the flow of the heat from the molten metal that is required to approximate the heat transference rate that is required in the sand mold designed for use in casting the same metal intended to be cast in the permanent mold. By the term "porous" I include all structures which are provided either with separated closed cells or with separated or connected passages, such as those which are commonly referred to by the term "cellular", "honeycomb", or "porous". Thus, one form of my improved permanent mold may consist of refractory material, such, for example, as porcelain clay, intimately mixed with a destructible substance. This mixture is forced into the desired shape of mold and it may be fired, or if not, then the first casting made therein will cause the destruction and removal of the other substance, producing a multiplicity of cells or openings in the mold and giving a porosity, the amount of which can be readily determined and varied by the amount of destructible material originally introduced into the mixture. Thereafter soft castings of uniform grain can be made repeatedly in this same mold.

Where greater strength is required than can be obtained by the use of a refractory material of the character referred to above, irregular metal particles, such as chips, borings, cuttings, shavings and the like may be formed into the desired mold shape, either alone or with a material such as sodium silicate, or magnesium chloride, for example, to act as a binder. If the metal particles are used alone they may be integrated or united in any suitable manner by incipient fusion on the contacting point or by heavy pressure to produce a single unitary structure of high strength and, by reason of the irregularity of shape of the particles, of considerable porosity, the latter characteristic being varied as desired by the type of shavings or chips that are employed. A porous metal structure may be produced by compressing together a mass of well mixed borings, turnings and metal

chips under very heavy pressure or this same mass of metal particles may be united by heating them to just the fusing temperature sufficient to cause a slight union between the contacting points or sides of the particles.

In the use of my permanent mold a parting or facing material may advantageously be employed on the inner surface of the mold in the same manner and for the same purpose as the same is now employed on sand molds, namely, to assist the flow of the metal, and to facilitate the removal of the casting. It will also be understood that while I have used the term "mold" throughout the present description, this term obviously includes both molds and what are commonly termed cores, but what are actually an inner mold introduced into the mold proper in some spaced relation to produce a hollow casting therebetween.

It will be apparent that the essential qualities or characteristics of the present mold are the considerable mechanical strength or bond between the particles originally employed to produce the mold and the capacity of transferring heat at a rate approximating that of a sand mold intended for the same casting. Various other compositions in addition to those already named may be employed to produce a mold having these characteristics. Thus, a refractory material such as porcelain clay, or metal particles with or without material such as clay, may be mixed with destructible material, such as sawdust, to produce a composition which, upon being raised to high temperature, will cause the destructible material to leave the mold, forming the required insulated openings or cells throughout the material. Or a cellular material may be employed in conjunction with a refractory material. Diatomaceous earth, which is itself cellular, may be mixed with metal particles or with metal particles and refractory material, or with refractory material alone, the porosity in this case being secured from the inherent characteristics of diatomaceous earth and, as in the previous cases, the porosity may be varied by the amount of diatomaceous earth employed.

It should be understood that the equivalent capacity for the transference of heat in the present mold as compared with that of sand molds is such capacity in operation. There is of course a certain difference in the operating conditions to which sand molds, and the present molds, will be subjected, since the present molds will be used repeatedly and without sufficiently long intervals between pourings to permit the mold to cool to the normal or room temperature of the foundry while ordinarily sand molds are at the atmospheric temperature of the foundry, although in certain cases sand molds may be heated but this is not the usual practice.

By the term "refractory", which has been used throughout the specification, I include

all materials which are refractory to the metal being cast. Thus, if metals of low melting point are being cast many substances, materials and other metals are refractory as regards that particular metal which would not be refractory if used with metals of high melting point, such for example, as iron or steel.

The present mold, whether formed of refractory material, such as a clay, refractory material and metal particles, or metal particles alone, is required to have the characteristic of a rate of heat transference approximating that of a sand mold for the same metal which is to be cast, and a strength sufficient to withstand the erosive and disintegrating effects of the wash of the molten metal thereagainst and the rapid and repeated sudden changes in temperature. This last characteristic is of course secured by the unitary or integrating condition of the material which forms the mold. The original particles or pieces of material which enter into the mold structure must be united with sufficient strength to resist the washing action of the metal as well as the disintegrating effect of the rapid temperature changes.

The field for the present invention is of course the entire foundry field wherever castings are produced rapidly, and particularly where the same casting is made over and over again, since under the latter circumstances immense savings can be effected by the use of the same mold and the avoidance of the labor and material necessary to reform the molds for each casting.

Other modes of applying the principle of my invention may be employed instead of the one explained, change being made as regards the composition herein disclosed, provided the ingredients or steps stated by any of the following claims or the equivalent of such stated ingredients or steps be employed.

I therefore particularly point out and distinctly claim as my invention:

1. A permanent porous mold for casting metal consisting of permanently united particles of metal having a rate of heat transference approximating that of a sand mold for the same casting operation and mechanical strength capable of repeatedly withstand-  
50 ing the erosive effect of the flow of molten metal thereagainst and the disintegrating action of repeated rapid changes of tempera-  
55 ture.

2. A permanent porous mold for casting metal consisting of permanently united particles of metal having an effective porosity in operation approximating that of sand molds for the same casting operation, and a me-  
60 chanical strength capable of repeatedly with-  
standing the erosive effect of the flow of molten metal thereagainst and the disinte-  
grating action of repeated rapid changes of  
65 temperature.

3. A permanent metal mold of unitary cel-  
lular structure, having a rate of heat trans-  
ference approximating that of a sand mold.

4. A permanent porous mold of unitary structure comprising united metal particles. 70  
Signed by me this 22d day of November,  
1927.

NELSON J. QUINN.

75

80

85

90

95

100

105

110

115

120

125

130